

Sept. 13, 1927.

1,642,359

D. CROESE

ELECTRIC FURNACE

Filed Dec. 1, 1926

2 Sheets-Sheet 1



Fig. 1.

Inventor.  
Dirk Croese,  
by Henry Black  
attorney

Sept. 13, 1927.

D. CROESE

1,642,359

ELECTRIC FURNACE

Filed Dec. 1, 1926

2 Sheets-Sheet 2



Inventor.  
Dish Croese,  
by Henry Blich  
Attorney

## UNITED STATES PATENT OFFICE.

DIRK CROESSE, OF LONDON, ENGLAND.

## ELECTRIC FURNACE.

Application filed December 1, 1926, Serial No. 152,020, and in Great Britain August 27, 1925.

This invention relates to the manufacture of metals and alloys from finely divided mineral substances and has particular reference to the production or reduction of metals from their ores in the electric furnace.

The object of the present invention is to provide an improved method of and means for the electric treatment of metal bearing substances in a finely divided state and which will enable such substances as iron-sand to be treated for the production of metal on a commercial scale.

According to the invention a process is provided for the production of metal or alloy from finely divided ores such as iron-sand, such process consisting in the removal of impurities, in causing the concentrated material to fall by gravity through a furnace divided into chambers in which the falling material is first preheated and is then caused to pass successively freely through a number of electric arcs under non-oxidizing conditions for the purpose of melting and reduction and in which further heat treatment is finally applied to facilitate separation of metal from slag.

The invention may be carried into effect in an electric furnace comprising a preheating chamber and a series of arc chambers through which the material to be treated falls freely by gravity, each arc chamber being provided with means to break up the falling material and deflect it on to the next arc of the series. The deflecting means preferably comprise a double cone of carbon disposed near the base of the arc chamber which tapers towards an outlet at its lower end and at the base of the series of chambers is disposed a heated crucible adapted to be tilted relatively to the upper part of the furnace or retort for the purpose of discharging molten metal or slag. Both retort and crucible are provided with means for preventing ingress of air during normal operation and whilst discharging and in order to render the reduction to metal as complete as possible the crucible may be heated by electric arcs in conjunction with a rotary, or otherwise movable magnetic field to ensure that the action of the arcs is made effective in every part of the crucible. Alternatively, the gases evolved by the reaction which takes place in the furnace and which are normally discharged to atmosphere or employed for power production may be utilized for heating the crucible.

Reference will now be made to the accompanying drawings which illustrate by way of example an electric furnace for carrying the invention into effect and in which:-

Figure 1 is a vertical sectional elevation of the furnace.

Figure 2 is a vertical sectional elevation of a tilting crucible adapted to be employed in conjunction with the furnace shown in Figure 1 and

Figure 3 is an external side elevation of the crucible shown in Figure 2.

The electric furnace 1 is of tubular form and comprises at the top a feed hopper 2 from the base of which a conveyor 3 removes the material to be treated to an inlet 4 disposed centrally at the top of the furnace 1, the conveyor 3 and inlet 4 being suitably housed within a casing 5 to prevent entry of air at the top of the furnace and avoid oxidization of the material under treatment. The incoming material which falls from the inlet passage 4 meets a conical baffle 6, the object of which is to break up and distribute the incoming finely divided material towards the furnace walls to prevent it passing too rapidly through the furnace and thus partially escaping treatment by the electric arcs as hereinafter described. The conical baffle 6 is disposed centrally within a preheating chamber 7 such baffle forming part of a double conical element supported on arms 8 projecting inwardly from a lining element 9 which forms the base of the preheating chamber and which tapers internally towards an outlet 10 at its base. The elements 6, 8 and 9 are formed from graphite or like material and are mounted in a lining of firebrick or like material 11 which forms the wall of the furnace and is enclosed by an outer sheathing of metal.

The upper or pre-heating chamber 7 of the furnace communicates through the outlet 10 with the first of a series of superimposed electrode chambers 12 each of which is of cylindrical form and is provided with a double conical baffle and a tapered base precisely similar in construction to those described above with reference to the preheating chamber.

Two or more electrodes 13 are disposed in each chamber 12 and are provided with the necessary devices for progressing them inwardly either automatically or manually as their ends become worn away. The walls of the furnace are provided at intervals in

- their height with a number of inspection doors fitted over openings 14 and preferably provided with transparent portions for sighting whilst each electrode chamber 12 is provided with a cleaning door fitted over an opening 15, the doors of openings 14 and 15 being luted with fire clay or hermetically sealed in some other manner prior to the furnace being set in operation.
- 10 The lowermost electrode chamber 12 is not provided with a tapered base but communicates directly with a crucible 16 disposed immediately below the base of the furnace, this crucible being arranged so that the 15 metal can separate from the slag and two or more separate outlets 17 and 18 are provided to enable the molten material to be withdrawn, these openings being normally closed by counterbalanced sliding doors 19. The 20 upper portion 20 of the crucible is of the same diameter as the lowermost electrode chamber 12 and the engagement between the two is by means of a pair of curved co-operating surfaces 21 which permit the crucible 25 to be tilted for the purpose of discharging. Whilst the furnace is in operation the base of the lowermost electrode chamber and the portion 20 of the crucible are coupled by means of a sleeve 22 which can be raised 30 when it is desired to tilt the crucible. The crucible 16 is provided with openings 23 at each side which enable three pairs of electrodes to be mounted within the crucible, this number being variable according to requirements in order to impart final treatment to the molten material which collects in the crucible. This final treatment may be conducted independently of the vertical furnace and dampers 24 and 25 slidably 35 mounted in the base of the lowermost electrode chamber and in the portion 20 of the crucible respectively may be provided to cut off communication between the vertical electrode chambers 12 and the crucible 16 40 when such final treatment is in progress. Beneath the crucible a framework 26 is provided to permit an electromagnet being mounted at this point for the purpose of attracting the arcs towards the surface of 45 the molten material collecting on the hearth 27 within the crucible and this electromagnet may be so arranged as to produce a rotating or otherwise movable magnetic field in order to ensure that the heating effect of 50 the arcs is carried to every part of the material collecting in the crucible.
- 55 The tilting mechanism for the crucible comprises a hand wheel 28 (see Figure 3) mounted on a spindle 29 and operating a worm 30 meshing with a worm wheel 31 with which a spur wheel 32 is co-axially mounted. The spur wheel 32 engages a toothed sector 33 fixed to the side of the crucible 16 and provided with a plane surface 34 struck from the same centre as the toothed sector 33 but engaged by friction rollers 35 for the purpose of braking the movement of the crucible when it is being moved towards the discharging position.
- 60 The furnace is provided with outlets 36 for waste gases such outlets communicating with chimneys 37 as shown in Figure 1. The ore to be treated is reduced to a finely divided condition by grinding or crushing and if ironsand is the substance to be treated 75 it is subject to a preliminary operation to remove impurities preferably by passage through a magnetic separating device. The process is then continued in the furnace above described in the following manner:— 80
- 85 The finely divided metal bearing material falls in a continuous stream from the inlet 4 into the furnace 1, the internal arrangement of which ensures that the falling particles are exposed to the heat generated by the arcs at the electrodes 13 for the length of time necessary to effect complete melting and reduction of all the material passed through the furnace. Whereas the melting point of titaniferous ironsand for example is 90 about 1500° C. and the temperature of the electric arc is over 3000° C. it follows that when ironsand is treated these particles will be completely melted and reduced by passage through the arcs, the arrangement of 95 which in addition to the construction of the furnace preclude the formation of a fused mass of material which has been an obstacle hitherto to the employment of the electric furnace in treating ironsand for the production of metal. It is to be noted that the up-100 most chamber 7 contains no electrodes but becomes heated to the degree necessary to preheat the falling material by part of the gases which ascend from the reaction 105 which takes place in the electrode chambers. The material resulting from the treatment in the furnace 1 collects in the crucible 16 where waste substances such as silica, lime and sulphur or phosphorus compounds collect in a layer above the layers of titanium and iron or steel. The waste gases from the reaction taking place within the furnace pass upwardly through the descending material and are withdrawn at a point below the pre-110 heating chamber through the outlets 36 and chimneys 37, part of these gases, however, circulating through the chamber 7 before escaping.
- 115 In an alternative arrangement the gas outlet conduit may pass to the base of the furnace where a draft of air is introduced and the gas burnt around the crucible 16 to maintain the contents thereof in a molten condition, this arrangement being employed as an alternative or in addition to the use of electrodes within the crucible as above described. If desired resistance heating may also be employed in addition to or in place 120 of the aforesaid methods of heating the 125 130

crucible. The gas conduit may further be provided with a branch leading to cooling and scrubbing apparatus from whence the gas may be passed into storage for use in operating a prime mover and an electricity generating plant.

The preheating chamber 7 may be heated electrically by elements disposed externally or internally thereof.

10 The conical elements 6 are preferably supported by four members 8 arranged at right angles one to the other so that the falling material is alternatively diverted into four streams and re-united in the outlet passages 15 10 so that a thorough separation of the material is obtained as it falls through each stage of the furnace ensuring that every particle receives the full influence of the electric arcs. The coned baffles also have the effect 20 of preventing clogging of the material and also of preventing the material passing too rapidly through the furnace.

When ironsand or other material containing or consisting of metallic oxide is under 25 treatment it may be mixed with a quantity of coke, anthracite, or other reducing agent before it is introduced to the feed hopper 2 or such reducing agent may be introduced to the crucible 16.

30 The treatment of ironsand by the process and in the furnace above described enables pure metal to be withdrawn from the crucible 16 through one of its outlets, and titanium slag at the other outlet, the metal being 35 a titanium steel alloy in which the percentage of titanium varies according to the length of time the treated material is maintained in a molten condition in the crucible. It has been found that some of the titanium always 40 goes into the slag which has thus various industrial applications, but by continued heating the titanium contents of the alloy can be reduced to less than 1 per cent producing the best quality titanium steel. If desired the 45 process above described may be carried out in an inert atmosphere, and for this purpose an inert gas would be introduced near the base of the lowermost electrode chamber 12.

The invention is not limited to any particular disposition of the electrodes within 50 each chamber 12 as the electrodes in one chamber may be disposed at a different angle relatively to those in the chamber above or below or several pairs of electrodes may be 55 disposed in each chamber.

Claims:

1. An electric furnace for the production of metals from their ores comprising a ver-

tical retort having a preheating chamber at the top and a series of arc chambers through 60 all of which chambers the material under treatment is caused to fall by gravity, a deflecting element disposed near the base of each chamber, a crucible in which the products from the retort collect, means for heating said crucible and means for preventing ingress of air to said crucible and retort.

2. An electric furnace for the production of metals from their ores comprising a vertical retort divided into separate chambers 70 by means of a number of double conical carbon baffles each of which co-operates with a downwardly tapering, throat of similar material, the upper chamber serving for pre-heating a stream of freely falling material 75 and the other chambers as arc chambers the base of said retort discharging into a heated crucible adapted to be tilted for the purpose of discharging molten metal and slag therefrom. 80

3. An electric arc furnace for treating finely divided ores comprising a preheating chamber, a series of arc chambers disposed vertically beneath said preheating chamber, a base to each arc chamber comprising an 85 inwardly tapering portion having inwardly directed members which support a double conical baffle concentrically with the chamber and form a number of passages through which the material deflected by the baffle is 90 caused to pass, means for feeding material to be treated to the top of said preheating chamber so as to fall by gravity through all of said chambers, and a heated crucible 95 adapted to receive the material treated in said chambers.

4. An electric arc furnace for treating finely divided ores comprising a preheating chamber, a series of arc chambers disposed vertically beneath said preheating chamber, 100 means for feeding material to said preheating chamber in such a manner that the operation is carried out under non-oxidizing conditions, a base to each arc chamber comprising an inwardly tapering portion having inwardly directed members which support a double conical baffle concentrically with the arc chamber and form a number of passages through which the material deflected by the baffle is caused to pass by gravity to the next 105 succeeding chamber, a heated crucible at the base of said furnace, means for shutting off the crucible from the furnace, and means for tilting the crucible for discharging purposes. 110

In witness whereof I affix my signature.  
DIRK CROESE.